

## UNITED STATES PATENT OFFICE.

CHARLES S. HOLLANDER, OF PHILADELPHIA, PENNSYLVANIA, ASSIGNOR TO ROHM & HAAS COMPANY, A CORPORATION OF DELAWARE.

## PREVENTION OF MARKING OFF.

No Drawing.

Application filed February 25, 1926. Serial No. 90,689.

In present-day practice, colored cotton 50 yarns dyed with dyes which are fast to alkali and chlorine bleach are woven with un-bleached cotton yarns. Later the entire 5 piece is subjected to a bleaching process which should not have any effect on the dyed yarns. This bleaching process involves two steps—first, a boiling out with caustic 10 soda or soda ash to remove waxes or other impurities from the raw cotton yarn; and second, a treatment with chlorine or hypo-chlorite solutions to remove the remaining 15 color.

Unfortunately in the first stage mentioned, 20 or as it is called, the "kier boil," it frequently happens that some of the color is transferred from the dyed yarn to the undyed portions of the piece goods, and this occurrence has been termed "marking off."

I have discovered that marking off may 25 be prevented by adding to the kier liquor a proper amount of a material which will either have a quinone-like structure in a hot or cold alkaline solution, or will be converted to a substance having such a structure when heated in an alkaline solution. To 30 the first group belong para-nitrosophenol, orthonitrosometacresol, benzoquinone, the naphthoquinones, etc.; and to the second group belong such products as paranitrosodimethylaniline and its hydrochloride. Paranitrosodimethylaniline, for example, is 35 converted into paranitrosophenol by boiling with alkali. All of these substances in both groups are intended to be embraced within the term "substances which show a quinone-like structure in a hot alkaline solution." Within this phrase I do not intend to include 40 higher substances such as those of the an-thracene series, as these themselves will dye the goods with a dye that will not be removed by the subsequent bleach. Inasmuch as substances such as the nitrosophenol or 45 nitrosocresol specified above will form sodium salts during the kier boiling operation, it is obvious that the salt itself may be used, if desired.

The amount of such substances to be used depends to a large extent on the concentra-

tion of alkali in the kier, the temperature 50 or pressure at which the goods are boiled, and also the length of time the goods are subjected to the treatment. The higher the concentration of alkali, the higher the temperature or pressure, and the longer the time 55 is the more of these substances has to be used, but some idea of the amount that may be used may be obtained from the following illustrative examples:

In these examples, unbleached cotton 60 goods with colored borders, dyed with various vat dyes, were rolled up tightly, and the roll was secured with a thread to prevent unrolling.

*First example.*—The roll of unbleached 65 cotton goods with vat dyed border was heated for two hours at 15 pounds pressure with twenty times its weight of water, 4% of caustic soda and 4% of orthonitrosometa-cresol. The goods were then unwrapped, 70 rinsed and bleached with sodium hypochlorite solution according to well-known procedure, and they showed a perfect white color without any markoff.

*Second example.*—A roll of unbleached 75 cotton goods with vat dyed borders was sub- jected to six hours boiling in an open vessel with 3% of caustic soda and 1% of nitroso-phenol and 2,000% of water. The goods were then aftertreated as before with the 80 same result.

*Third example.*—Another roll of un- 85 bleached cotton goods with vat dyed pattern was boiled with 4% of caustic and 5 1/3% of paranitrosodimethylaniline hydrochloride, and enough water to submerge the goods for three hours at 15 pounds pressure. The goods were then also subjected to the same aftertreatment with the same result.

It is to be understood that these examples 90 are given by way of illustration only, and that the temperatures, time of treatment, and concentration, that is, the relative amounts of water and chemicals used, may be varied within wide limits without de- 95 parting from the spirit of my invention.

What I claim is:

1. In the art of bleaching fabrics which

include vegetable yarns dyed with dyes fast to alkali and chlorine bleach, the step of subjecting the goods to the action of a hot alkaline solution comprising a substance having not more than two benzene nuclei which in a hot alkaline solution will show a quinone-like structure.

2. A process as defined in the foregoing claim in which the said substance comprised in the alkaline solution will show a quinone-like structure in a cold alkaline solution as well as in a hot alkaline solution. <sup>10</sup>

CHARLES S. HOLLANDER.